

## UNITED STATES PATENT OFFICE

FRANCO BANDINI, OF ROME, ITALY

BRICK MAKING PROCESS IN WHICH QUICK DRYING AND BURNING ARE COMBINED IN  
A SINGLE OPERATION

No Drawing. Application filed August 5, 1930, Serial No. 473,290, and in Italy July 12, 1930.

As is publicly known, the ordinary process for brick making is the following.

Brick clay when coming from the quarry is first conveniently prepared so as to acquire, by eventually adding a suitable quantity of water the necessary degree of plasticity. The mixture thus formed is sent to the brick moulding machines, the moulded bricks obtained being then naturally or artificially dried. The dried bricks are subsequently burnt in a furnace and extracted when burning is completed and after cooling.

All this requires a long time and a remarkable number of operations which owing to the intrinsic low value of the material treated, considerably increase the cost of the final product.

In order to avoid said inconveniences, that is to say in order

(a) to reduce to the minimum the time required for drying, and in order to

(b) combine into a single operation quick drying and burning without any interruption in the process.

The method according to application has been studied and practically tried for testing the good quality of the product obtained.

The process comprises the following steps:

1. The mixture of clay is heated before moulding to about 95° C. and moulded by a press or drawing moulding machine, the heating being continued during moulding, a greater plasticity of the clay and a subsequent economy in the driving power required by the moulding machine being thus obtained.

2. After moulding, the brick is placed in a refractory box on the bottom of which a layer of sand or other powdery substance has been previously arranged, this sand or the like being also preheated to the temperature of nearly 95° C.

3. The brick is then completely covered with more warm sand previously mixed with a convenient quantity of powdery fuel. Liquid fuel may be also used instead of powdery fuel, this use in any case not being excluded.

4. The refractory box is introduced into a

tunnel of such a length that after arranging in a convenient determined position a heat source, a temperature of nearly 95° C. is obtained at the inlet opening of the tunnel, this temperature of course increasing progressively from the inlet opening of the tunnel towards the point where the heat source mentioned has been arranged, this source having the necessary intensity to produce the ignition of the fuel mixed with sand contained in the refractory box when this box reaches the position of said heat source.

5. The length of tunnel is such that at the outlet opening the temperature is nearly the same as that of the external air.

It is clear then that if the refractory box is run with a convenient speed within and along the tunnel the brick contained in the box successively takes the different temperatures met on the way from the initial one of 95° C. to that of the external air passing through the temperature produced by the heat source destined to the ignition of the fuel contained in the refractory box.

This combustion lasts till consumption of fuel, this fuel being dosed in such a way as to obtain the drying and burning of the brick contained in the box.

Practically the total quantity of fuel necessary for drying and burning bricks is, as known, about the 6% of the weight of the bricks.

After consumption of the fuel the refractory box proceeding along the tunnel yields its heat to the air flowing in through the outlet opening, so that said box with the material contained therein will have about the same temperature as the external air.

It is clear that if, after the first box, more boxes filled in the same manner are introduced in the tunnel, each of them will have, in each portion of this tunnel the same temperature as that assumed in said portion by the first box. When working conditions have been reached, that is when in each section of the tunnel the temperature is constant the functioning of the external heat source may be suppressed, the ignition of

the fuel being produced by the rise of temperature of the box.

According to numerous accurate trials the time required for drying, burning and subsequently cooling bricks according to the process specified is a little more than 36 hours. This time, as is well known is not at all sufficient according to the systems presently used, not even for obtaining the 10 artificial drying of bricks.

It is important to remark that the process of bricks making according to application may be carried out in practice even without mixing powdery or liquid fuel with sand, 15 provided a convenient external heat source is at disposal, of a sufficient intensity for producing the necessary temperature for working conditions.

It is also possible to reduce the quantity 20 of powdery or liquid fuel mixed with sand but by keeping at the same time in action an external heat source, though with a reduced emission of heat.

The process according to application may 25 also be used for making bricks, the clay employed being previously dried and finely ground, then subjected to a convenient pressure within stamping forms, the invention being adapted for dry brick making.

30 The process may also be employed when bricks are moulded cold with a drawing machine, the mixture of clay used being cold, then immersed in a cold bed of sand and fuel. Of course the bricks might also be 35 drawn warm and immersed in a cold bed or drawn cold and immersed in a warm bed of sand and fuel.

Having now particularly described and 40 ascertained the nature of my said invention and in what manner the same is to be performed, I declare that what I claim is:

1. A process of making molded ceramic articles by drying and burning in one operation in one apparatus, which comprises 45 pre-heating suitable clay mixture, then molding articles from said mixture during continued heating, then inserting such molded articles in a bed consisting of sand and powdery fuel preheated to the same 50 temperature as said articles and contained in a refractory box and completely covered by sand of the same temperature; then successively introducing such filled boxes in a tunnel-oven having the same temperature 55 at the inlet as said articles and drying and burning said molded articles therein by means of the fuel in the bed while slowly passing the filled boxes through the oven.

60 2. A process according to claim 1, in which the molding is effected at a temperature of about 95° C. with the aid of the preheated molding material.

65 3. A process according to claim 1 in which the temperature is uniformly maintained during the process at about 95° C.

until the articles enter the inlet opening of the tunnel-oven where the heat intensity is gradually increased to ignite said fuel.

4. A process according to claim 1 in which the temperature is uniformly maintained during the process at about 95° C. 70 until the articles enter the inlet opening of the tunnel-oven where the heat intensity is gradually increased to about 300° C. to ignite said fuel. 75

In testimony whereof I have hereunto signed my name.

FRANCO BANDINI.

80

85

90

95

100

105

110

115

120

125

130